

# United States Patent [19]

Singer

[11] Patent Number: **4,619,884**

[45] Date of Patent: **Oct. 28, 1986**

- [54] **PHOTOGRAPHIC PRODUCTS EMPLOYING NONDIFFUSIBLE N',N'-DIAROMATIC CARBOCYCLIC—OR DIAROMATIC HETEROCYCLIC—SULFONOHYDRAZIDE COMPOUNDS CAPABLE OF RELEASING PHOTOGRAPHICALLY USEFUL GROUPS**
- [75] Inventor: Stephen P. Singer, Rochester, N.Y.
- [73] Assignee: Eastman Kodak Company, Rochester, N.Y.
- [21] Appl. No.: **759,786**
- [22] Filed: **Jul. 29, 1985**
- [51] Int. Cl.<sup>4</sup> ..... G03C 1/40; G03C 5/54; G03C 1/34; G03C 1/42
- [52] U.S. Cl. ..... 430/223; 430/212; 430/217; 430/218; 430/219; 430/542; 430/543; 430/559; 430/562; 430/564; 430/566; 430/591; 430/598; 430/600; 430/603; 430/606; 430/611; 430/621; 430/955; 430/957; 430/959
- [58] Field of Search ..... 430/955-960, 430/505, 544, 564, 562, 551, 550, 606, 607, 611, 613, 621, 223, 218, 559, 219, 543, 566, 598, 603, 600, 212, 542, 217, 591

- [56] **References Cited**
- U.S. PATENT DOCUMENTS**
- 4,278,748 7/1981 Sidhu et al. ..... 430/598  
4,369,243 1/1983 Credner et al. ..... 430/223  
4,430,420 2/1984 Adin ..... 430/619

## OTHER PUBLICATIONS

- Research Disclosure, May 1977, #15776, pp. 67-68.  
Research Disclosure, Oct. 1978, #17465, p. 64.  
Research Disclosure, vol. 128, Dec. 1974, Item No. 12823, pp. 22 to 25 (Application p. 1, lines 25-26).

Primary Examiner—Richard L. Schilling  
Attorney, Agent, or Firm—Thomas F. Kirchoff

## [57] ABSTRACT

Photographic elements and assemblages are described which employ nondiffusible N',N'-diaromatic carbocyclic—or diaromatic heterocyclic—sulfonohydrazide compounds which are capable of releasing photographically useful groups in an imagewise manner as a function of silver halide development.

13 Claims, No Drawings

PHOTOGRAPHIC PRODUCTS EMPLOYING  
NONDIFFUSIBLE N',N'-DIAROMATIC  
CARBOCYCLIC—OR DIAROMATIC  
HETEROAROMATIC—SULFONOHYDRAZIDE  
COMPOUNDS CAPABLE OF RELEASING  
PHOTOGRAPHICALLY USEFUL GROUPS

This invention relates to photography and more particularly to color diffusion transfer photography employing novel nondiffusible sulfonohydrazide compounds capable of releasing diffusible photographically useful groups.

The release of diffusible photographically useful groups from nondiffusible compounds is well known in photographic technology. However, the manner of releasing a desired group is only a part of the overall consideration. Some released groups fall short of providing properties which are required to assure acceptable photographic image quality, particularly in color diffusion transfer processes.

U.S. Pat. No. 4,369,243 describes sulfilimine compounds which release diffusible photographically active moieties. Investigation of these compounds reveals that although an acceptable rate of dye release can be obtained the resulting images have less than acceptable sensitometric properties, in particular, low D<sub>max</sub> and high D<sub>min</sub> values.

*Research Disclosure*, Volume 128, December 1974, Item 12823, pages 22 to 25, describes sulfohydrazide dye-releasing compounds for photographic color diffusion transfer use. These compounds release a dye moiety as a result of rupturing a sulfur-nitrogen bond so that the released dye moiety has a free SO<sub>3</sub><sup>-</sup> radical attached thereto which imparts very high solubility to the released dye in alkaline media.

Attempted use of dyes having free sulfonic acid radicals in alkaline environment has been less than satisfactory due to a tendency toward image smearing. It is believed this smearing problem is caused by the high solubility of such dyes in the alkaline environment encountered in color diffusion transfer processing. This solubility leads to rapid diffusion of released dyes in all directions in a photographic recording material. This rapid diffusion, and resulting smearing, renders the dyes unacceptable for commercial use.

Accordingly, it is desirable to provide a nondiffusible compound capable of rapid and efficient release of a photographically useful group, as a function of silver halide development, in color diffusion transfer photographic elements and assemblages, which group will provide acceptable photographic properties.

One embodiment of this invention provides a photographic element comprising a support having thereon at least one photosensitive silver halide emulsion layer having associated therewith a nondiffusible N',N'-diaromatic carbocyclic- or diaromatic heterocyclic-sulfonohydrazide compound capable of releasing a diffusible photographically useful group, or precursor thereof, wherein at least one of said aromatic groups comprises a nitro substituent in the 2- position or in a position conjugated thereto.

In a preferred embodiment of this invention the N',N'-di-aromatic carbocyclic- or diaromatic heterocyclic-sulfonohydrazide compound is represented by the structural formula:



where

each Z independently represents the atoms necessary to complete a substituted or an unsubstituted one- or a two-ring carbocyclic or heterocyclic group containing 5 to 7 nuclear atoms in each ring;

J is a nitro group substituted in the 2- position or in a position conjugated thereto;

m and n are each integers of 0, 1 or 2 with the proviso that either m or n is at least 1;

R is hydrogen or an alkyl group having from 1 to about 6 carbon atoms; and

PUG is a photographically useful group.

The type of rings which Z can complete include, for example, benzene, pyridine, diazine, naphthalene, quinoline, furan, thiophene, pyrrole, isoxazole, benzofuran, benzothiophuran, indole, indene and azulene.

As noted above, Z can represent the atoms necessary to complete a substituted or an unsubstituted one- or two-ring carbocyclic or heterocyclic group containing 5 to 7 nuclear atoms in each ring. Substituents, other than one or more nitro groups as defined above for J, can include a straight or branched chain alkyl or alkoxy group having from 1 to about 30 carbon atoms; an aryl group having from 6 to about 30 carbon atoms; one or more halogen atoms, for example, chloro, bromo, iodo or fluoro; cyano; a carbamoyl group having the formula —CON(R<sup>2</sup>)<sub>2</sub> or a sulfamoyl group having the formula —SO<sub>2</sub>N(R<sup>2</sup>)<sub>2</sub>, where each R<sup>2</sup> independently represents a hydrogen atom; an alkyl or an alkoxy group having from 1 to about 30 carbon atoms or an aryl or an aryl oxy group having from 6 to about 30 carbon atoms.

Reference to nondiffusibility of the N',N'-di-aromatic carbocyclic- or diaromatic heterocyclic-sulfonohydrazide compound is intended to mean that the compound is not free to diffuse out of the layer in which it is coated. Nondiffusibility is a property of the hydrazide compound under both acidic and alkaline conditions, including highly alkaline conditions such as are encountered in a color diffusion transfer processing environment.

Nondiffusibility is commonly imparted to compounds which release photographically useful groups by use of a ballast group substituted on at least one of the carbocyclic or heterocyclic rings completed by Z. The type of ballast group used is not critical so long as it confers the desired nondiffusibility property to the compound. Typical ballast groups include long-chain alkyl radicals, as well as aromatic radicals of the benzene and naphthalene series. Such groups can be linked directly to the carbocyclic or heterocyclic rings completed by Z. Useful ballast groups generally have at least 8 carbon atoms although satisfactory ballasting can be obtained with two or more smaller groups, such as two t-amyl groups. Ballast groups include substituted or unsubstituted alkyl groups having up to about 30 carbon atoms, carbamoyl radicals, having up to about 30 carbon atoms, such as —CONH(CH<sub>2</sub>)<sub>4</sub>—O—C<sub>6</sub>H<sub>3</sub>(C<sub>5</sub>H<sub>11</sub>)<sub>2</sub> or

—CON(C<sub>12</sub>H<sub>25</sub>)<sub>2</sub>, or keto radicals having up to about 30 carbon atoms, such as —CO—C<sub>17</sub>H<sub>35</sub> or —CO—C<sub>6</sub>H<sub>4</sub>(—C<sub>12</sub>H<sub>25</sub>).

Specific examples of ballast groups useful in this invention are described in the November 1976 edition of *Research Disclosure*, pages 68 through 74, and in the April 1977 edition of *Research Disclosure*, pages 32 through 39, the disclosures of which are hereby incorporated by reference.

The photographically useful group (PUG) released by the compounds of this invention can be any group which is desirably made available in a photographic element in an imagewise fashion. The PUG can be an image dye or an image dye precursor. Dye or dye precursor moieties released from the compounds of this invention can include dyes already well known in the art which are suitable for image transfer applications. These dyes or dye precursors are disclosed in one or more of U.S. Pat. Nos. 3,230,085; 3,307,947; 3,579,334 and 3,684,513, and also include the phenylazonaphthyl dyes of U.S. Pat. Nos. 3,929,760; 3,931,144; 3,932,380; 3,932,381; 3,942,987; 3,954,476; 4,001,204 and 4,013,635; the phenylazopyrazoline dyes of U.S. Pat. No. 4,013,633; the arylazopyrazolotriazole and arylazopyridinol dyes of U.S. Pat. No. 4,142,891; the arylazo dyes of U.S. Pat. No. 4,156,609; the pyridylazopyrazole and pyrimidylazopyrazole dyes of U.S. Pat. No. 4,148,641; the pyridylazonaphthol dyes of U.S. Pat. No. 4,147,544; the arylazoisouquinolinol dyes of U.S. Pat. No. 4,186,642; and the arylazovinylol dyes of U.S. Pat. No. 4,148,643. Such dyes have good stability and exhibit good diffusion under conditions of color transfer usage. They are also compatible with known and commonly used mordants.

PUG can also be a photographic reagent, that is a moiety which, upon release from a compound of this invention, undergoes a reaction with components in the described photographic elements or assemblages. Photographic reagents which can be released by the compounds of this invention include development inhibitors, development accelerators, bleach inhibitors, bleach accelerators, couplers, developing agents, silver complexing agents, fixing agents, toning agents, hardening agents, tanning agents, fogging agents, antifogging agents and chemical or spectral sensitizing or desensitizing agents.

PUG's which form development inhibitors upon release from the compounds of this invention can be of any type known in the art. These include the development inhibitors described in U.S. Pat. Nos. 3,227,554; 3,384,657; 3,615,506; 3,617,291 and 3,733,201 and in U.K. Patent No. 1,450,479, the disclosures of which are incorporated herein by reference. Preferred development inhibitors are iodide and heterocyclic compounds such as mercaptotetrazoles, selenotetrazoles, mercaptobenzothiazoles, mercaptobenzimidazoles, seleneobenzimidazoles, benzotriazoles and benzodiazoles. Structures of preferred development inhibitor moieties are:



where R<sup>3</sup> is hydrogen alkyl of 1 to 8 carbon atoms (e.g. methyl, ethyl, butyl), phenyl or substituted phenyl and R<sup>4</sup> is hydrogen or one or more halogen atoms (e.g. chloro, fluoro, bromo or iodo), lower alkyl of 1 to 4 atoms or nitro groups.

The compounds of this invention are useful in positive-working image transfer systems. For example, where the released photographically useful group is a dye image-forming compound, a positive dye image is produced which is inverse to the development of silver halide. In a system of this type the more versatile and conventional negative silver halide emulsions can be used.

Representative nitrodiaromatic-substituted sulfonohydrazide compounds useful in this invention include:

WHERE PUG IS AN IMAGE DYE OR AN IMAGE  
DYE PRECURSOR



-continued

6.



7.



8.



9



10.



-continued



11.



12.



13



## WHERE PUG IS A PHOTOGRAPHIC REAGENT OR A PHOTOGRAPHIC REAGENT PRECURSOR 50



14



$R^3$ =Hydrogen or a hydrolyzable group such as



where  $R^4$  is alkyl having from 1 to 18 carbon atoms or aryl having from 6 to 18 carbon atoms.

A preferred embodiment of the present invention comprises a photographic element comprising a support having thereon a red-sensitive silver halide emulsion

layer having associated therewith an N',N'-di-aromatic carbocyclic- or diaromatic heterocyclic-sulfonohydrazide compound of this invention which is capable of releasing a cyan image dye-providing moiety, a green-sensitive silver halide emulsion layer having associated therewith an N',N'-di-aromatic carbocyclic- or diaromatic heterocyclic-sulfonohydrazide compound of this invention which is capable of releasing a magenta image dye-providing moiety and a blue-sensitive silver halide emulsion layer having associated therewith an N',N'-di-aromatic carbocyclic- or diaromatic heterocyclic-sulfonohydrazide compound of this invention which is capable of releasing a yellow image dye-providing moiety.

A photographic assemblage in accordance with this invention comprises:

- (a) a photographic element comprising a support having thereon at least one photosensitive silver halide emulsion layer having associated therewith a nondiffusible N',N'-di-aromatic carbocyclic- or diaromatic heterocyclic-sulfonohydrazide compound capable of releasing a photographically useful group or precursor thereof, wherein at least one of said aryl groups comprises a nitro substituent in the 2- position or in a position conjugated thereto;
  - (b) a dye image-receiving layer; and
  - (c) an alkaline processing composition with means for discharging same within said assemblage;
- said assemblage also comprising a silver halide developing agent.

The processing composition may be inserted into the assemblage by interjecting processing solution with communicating members similar to hypodermic syringes which are attached either to a camera or camera cartridge. The processing composition can also be applied by means of a swab or by dipping into a bath. Another method of applying processing composition in the assemblage is the liquid spreading means described in U.S. Pat. No. 4,370,407.

The assemblage itself preferably contains the alkaline processing composition and means containing same for discharge within the assemblage. There can be employed, for example, a rupturable container which is adapted to be positioned during processing so that a compressive force applied to the container by pressure-applying members, such as would be found in a camera designed for in-camera processing, will effect a discharge of the container's contents within the assemblage.

Image-receiving layers which can be employed in the photographic assemblages of this invention can be any of those recognized in the art as providing the desired functions of mordanting or otherwise fixing the dye images. The choice of mordant will, at least in part, depend upon the dye to be mordanted and can be a basic polymeric mordant, such as described in U.S. Pat. Nos. 2,882,156; 3,625,694; 3,709,690; 3,898,088; 3,958,995; 3,859,096; or in the November 1976 edition of Research Disclosure, pages 80-82.

The dye image-receiving layer in the above-described assemblage is optionally located on a separate support adapted to be superposed on the photographic element after exposure thereof. Such an image-receiving element is generally disclosed in U.S. Pat. No. 3,362,819. When the means for discharging processing composition is a rupturable container, it is usually positioned in relation to the photographic element and the image-receiving layer so that a compressive force applied to

the container by pressure-applying members, such as would be found in a typical camera used for in-camera processing, will effect a discharge of the container's contents between the image-receiving layer and the outermost layer of the photographic element. After processing, the dye image-receiving layer is separated from the photographic element.

The dye image-receiving layer in the above-described assemblage in another embodiment is located integrally with the photographic element between the support and the lowermost photosensitive silver halide emulsion layer. One useful format for integral receiver-negative photographic elements is disclosed in Belgian Patent No. 757,960. In such an embodiment, the support for the photographic element is transparent and is coated with an image-receiving layer, a substantially opaque light-reflective layer, e.g., TiO<sub>2</sub>, and then the photosensitive layer or layers described above. After exposure of the photographic element, a rupturable container containing an alkaline processing composition and an opaque process sheet are brought into superposed position. Pressure-applying members in the camera rupture the container and spread processing composition over the photographic element as the film unit is withdrawn from the camera. The processing composition develops each exposed silver halide emulsion layer and dye images are formed as a function of development which diffuse to the image-receiving layer to provide a positive, right-reading image which is viewed through the transparent support on the opaque reflecting layer background. For other details concerning the format of this particular integral film unit, reference is made to the above-mentioned Belgian Patent No. 757,960.

Another format for integral negative-receiver photographic elements in which the present invention is useful is disclosed in Canadian Patent No. 928,559. In this embodiment, the support for the photographic element is transparent and is coated with the image-receiving layer, a substantially opaque, light-reflective layer and the photosensitive layer or layers described above. A rupturable container containing an alkaline processing composition and an opacifier is positioned adjacent the top layer and a transparent top sheet which has thereon a neutralizing layer and a timing layer. The film unit is placed in a camera, exposed through the transparent top sheet and then passed through a pair of pressure-applying members in the camera as it is being removed therefrom. The pressure-applying members rupture the container and spread processing composition and opacifier over the negative portion of the film unit to render it light-insensitive. The processing composition develops each silver halide layer and dye images, formed as a result of development, diffuse to the image-receiving layer to provide positive, right-reading images which are viewed through the transparent support on the opaque reflecting layer background. For further details concerning the format of this particular integral film unit, reference is made to the above-mentioned Canadian Patent No. 928,559.

Still other useful integral formats in which this invention can be employed are described in U.S. Pat. Nos. 3,415,644; 3,415,645; 3,415,646; 3,647,437 and 3,635,707. In most of these formats, a photosensitive silver halide emulsion is coated on an opaque support and a dye image-receiving layer is located on a separate transparent support superposed over the layer outermost from the opaque support. In addition, this transparent sup-

port also preferably contains a neutralizing layer and a timing layer underneath the dye image-receiving layer.

A preferred photographic assemblage in accordance with the invention comprises:

(a) a photographic element comprising a support having thereon the following layers in sequence: a dye image-receiving layer, a stripping layer, a substantially opaque layer and a photosensitive silver halide emulsion layer having associated therewith a dye image-providing compound as described above;

(b) a transparent cover sheet superposed over the silver halide emulsion layer; and

(c) an opaque alkaline processing composition and means containing same for discharge, during processing, between the cover sheet and the photosensitive element.

Any material may be employed as the stripping layer in the photographic assemblage described above provided it will perform the desired function of cleanly stripping. Such materials are disclosed, for example in U.S. Pat. Nos. 3,220,835; 3,730,718 and 3,820,999 and include gum arabic, sodium alginate, pectin, polyvinyl alcohol and hydroxyethyl cellulose. Hydroxyethyl cellulose is preferably employed as the stripping layer.

The stripping layer materials employed in the assemblage described above can be employed in any amount which is effective for the intended purpose. Good results are obtained at a concentration of from about 5 to about 2000 mg/m<sup>2</sup> of element. The particular amount to be employed will vary depending on the particular stripping layer material employed and the nature of the other layers of the diffusion transfer element.

The concentration of compound that is employed in the present invention to release a PUG may be varied over a wide range, depending upon the particular PUG sought to be released and the results which are desired. For example, where an image dye or image dye-precursor is desired, a compound of the present invention may be coated in a silver halide emulsion layer or in a layer adjacent thereto. Coating can be accomplished by using a solution containing between about 0.5 and about 8 percent by weight of the compound distributed in a hydrophilic film-forming natural material or synthetic polymer, such as gelatin, polyvinyl alcohol, etc., which can be permeated by aqueous alkaline processing com-

position.

Where the PUG to be released is other than an image dye or dye-providing compound, the compounds of this invention containing such PUG may be utilized in various layers of the described photographic element and in varying concentrations to ensure release of the desired amount of PUG.

The photographic element described above can be treated in any manner with an alkaline processing composition to effect or initiate development. A preferred method for applying processing composition is by use of a rupturable container or pod which contains the composition. In general, the processing composition contains a developing agent, although the composition could be an alkaline solution with the developing agent being incorporated in the photographic element or cover sheet. In the latter case the alkaline solution serves to activate the incorporated developer.

A variety of silver halide developing agents or electron transfer agents (ETA's) are useful in this invention. In certain embodiments of the invention, any ETA can be employed as long as it cross-oxidizes with the dye-providing compounds described herein. The ETA may

also be incorporated in the photosensitive element to be activated by the alkaline processing composition. Specific examples of ETA's useful in this invention include hydroquinone compounds, catechol compounds, and

5 3-pyrazolidinone compounds as disclosed in column 16 of U.S. Pat. No. 4,358,527. A combination of different ETA's, such as those disclosed in U.S. Pat. No. 3,039,869, can also be employed. These ETA's are employed in the liquid processing composition or contained, at least in part, in any layer or layers of the photographic element or assemblage to be activated by the alkaline processing composition, such as in a silver halide emulsion layer, a separate dye image-providing compound layer, an interlayer or an image-receiving layer.

In a preferred embodiment of the invention, the silver halide developer or ETA employed becomes oxidized upon development and reduces silver halide to silver metal. The oxidized developer then cross-oxidizes the compound of this invention. The product of cross-oxidation then undergoes alkaline hydrolysis, thus releasing an imagewise distribution of PUG which is then free to diffuse through the photographic element to provide the desired result.

Release of the PUG occurs as a result of rupturing the bond between the two nitrogen atoms of the N',N'-diaromatic carbocyclic- or diaromatic heterocyclic-sulfonohydrazide compound. The released PUG moiety has attached thereto the —NR—SO<sub>2</sub>— fragment which, due to its solubility in alkaline media, facilitates diffusion of the released PUG in the photographic element during processing.

In using the compounds according to the invention which release diffusible dyes as a function of development, either conventional negative-working or direct-positive silver halide emulsions are employed. If the silver halide emulsion employed is a conventional negative-working emulsion a positive image will be obtained in the image-receiving layer. Use of a direct-positive emulsion will produce a negative image in the image-receiving layer. Such a negative can be used to produce positive prints.

The film unit or assemblage of this invention can be used to produce positive images in single or multicolors, when used in a three-color system, each silver halide emulsion layer will have associated therewith a compound capable of releasing a PUG which is an image dye, or image dye precursor, which has a predominant spectral absorption within the region of the visible spectrum to which said silver halide emulsion is sensitive. The compound which releases the dye, or dye precursor, is contained either in the silver halide emulsion layer or in a layer contiguous thereto.

The various silver halide emulsion layers of a color film assemblage employed in this invention are generally disposed in the usual order, i.e., the blue-sensitive silver halide emulsion layer first with respect to the exposure side, followed by the green-sensitive and red-sensitive silver halide emulsion layers. If desired, a yellow dye layer or a yellow colloidal silver layer can be present between the blue-sensitive and green-sensitive silver halide emulsion layers for absorbing or filtering blue radiation that is transmitted through the blue-sensitive layer. If desired, the selectively sensitized silver halide emulsion layers can be disposed in a different order, e.g., the blue-sensitive layer first with respect to the exposure side, followed by the red-sensitive and green-sensitive layers.

The rupturable container employed in certain embodiments of this invention is disclosed in U.S. Pat. Nos. 2,543,181; 2,643,886; 3,653,732; 2,723,051; 3,056,492; 3,056,491 and 3,152,515. Such containers usually comprise a rectangular sheet of fluid-and-air-impervious material folded longitudinally upon itself to form two walls which are sealed to one another along their longitudinal and end margins to form a cavity in which processing composition is contained.

Except where noted otherwise, the silver halide emulsion layers employed in the invention comprise photosensitive silver halide dispersed in gelatin along with the dye-providing compounds.

Scavengers for oxidized developing agent can be employed in various interlayers of the photographic elements of the invention. Suitable materials are disclosed on page 83 of the November 1976 edition of *Research Disclosure*, the disclosure of which is hereby incorporated by reference.

Use of a neutralizing material in photographic elements of this invention will usually increase the stability of the transferred image since it will effect a reduction in the pH of the image layer from about 13 or 14 to at least 11, and preferably 5 to 8, within a short time after imbibition. Suitable materials and their functioning are disclosed on pages 22 and 23 of the July 1974 edition of *Research Disclosure*, and pages 35 through 37 of the July 1975 edition of *Research Disclosure*, the disclosures of which are hereby incorporated by reference.

A timing or inert spacer layer can be employed over the neutralizing layer which "times" or controls the pH reduction as a function of the rate at which alkali diffuses through the inert spacer layer. Examples of such timing layers and their functioning are disclosed in the *Research Disclosure* articles mentioned in the paragraph above concerning neutralizing layers.

The alkaline processing composition employed in this invention is the conventional aqueous solution of an alkaline material, e.g., alkali metal hydroxides or carbonates such as sodium hydroxide, sodium carbonate or an amine such as diethylamine, preferably possessing a pH in excess of 11, and preferably containing a developing agent as described previously. Suitable materials and addenda frequently added to such compositions are disclosed on pages 79 and 80 of the November 1976 edition of *Research Disclosure*, the disclosure of which is hereby incorporated by reference.

The alkaline solution-permeable, substantially opaque, light-reflective layer employed in certain embodiments of photographic assemblages used in this invention is described more fully in the November 1976 edition of *Research Disclosure*, page 82, the disclosure of which is hereby incorporated by reference.

The supports for the photographic elements used in this invention can be any material as long as it does not deleteriously affect photographic properties and is dimensionally stable. Typical flexible sheet materials are described on page 85 of the November 1976 edition of *Research Disclosure*, the disclosure of which is hereby incorporated by reference. The supports may be either opaque for obtaining a reflection print or clear or semi-translucent for obtaining a transparency. If transparent

cies are obtained, they may be viewed through the support side or the opposite side depending upon the "viewing" required.

The silver halide emulsions useful in this invention are well known to those skilled in the art. They are described in *Research Disclosure*, Volume 176, December 1978, Item No. 17643, pages 22 and 23, "Emulsion preparation and types", and are usually chemically and spectrally sensitized as described on page 23, "Chemical sensitization", and "Spectral sensitization and desensitization", of the above article; they are optionally protected against the production of fog and stabilized against loss of sensitivity during keeping by employing the materials described on pages 24 and 25, "Antifogants and stabilizers", of the above article; they usually contain hardeners and coating aids as described on page 26, "Hardeners", and pages 26 and 27, "Coating aids", of the above article; they and other layers in the photographic elements used in this invention usually contain plasticizers, vehicles and filter dyes described on page 27, "Plasticizers and lubricants"; page 26, "Vehicles and vehicle extenders"; and pages 25 and 26, "Absorbing and scattering materials", of the above article; they and other layers in the photographic elements used in this invention can contain addenda which are incorporated by using the procedures described on page 27, "Methods of addition", of the above article; and they are usually coated and dried by using the various techniques described on pages 27 and 28, "Coating and drying procedures", of the above article, the disclosures of which are hereby incorporated by reference.

The term "nondiffusing" used herein has the meaning commonly applied to the term in photography and denotes materials that for all practical purposes do not migrate or wander through organic colloid layers such as gelatin in an alkaline medium, in the photographic elements of the invention and preferably when processed in a medium having a pH of 11 or greater. The same meaning is to be attached to the term "immobile". The term "diffusible" as used herein has the converse meaning and denotes materials having the property of diffusing effectively through the colloid layers of the photographic elements in an alkaline medium in the presence of "nondiffusing" materials. "Mobile" has the same meaning.

The term "associated therewith" as used herein is intended to mean that the materials can be in either the same or different layers so long as the materials are accessible to one another.

The nitro diaryl-substituted redox dye releasing (RDR) compounds of this invention can be synthesized either by reaction of an aldehyde hydrazone, such as benzaldehyde, 1-naphthaldehyde or picolinaldehyde (Synthesis 1, below), or from a nitrosubstituted aromatic amine, such as p-nitroaniline (Synthesis 2, below).

#### Synthesis 1

The schematic representation presented below describes the preparation of positive RDR Compound No. 1, wherein the PUG which is released is a magenta dye:



25

**Synthesis of the benzylhydrazone:**

m-Hexadecyloxyphenol (7.5 g, 22.4 mmol) was added in small portions to a 50 percent sodium hydroxide dispersion, (1.2 g, 25 mmol) in toluene (100 ml) under nitrogen. After 20 minutes, the resulting suspension was cooled and a solution of p-nitrophenylbenzylhydrazone bromide (5 g, 15.6 mmol)\* in 30 ml tetrahydrofuran was added dropwise. After 4 hours at room temperature (22° C.), the reaction was extracted with ether, washed with 10 percent hydrochloric acid and dried with anhydrous magnesium sulfate. After filtering, the solvents were removed and the resulting solid was purified by silica gel column chromatography eluting with dichloromethane/cyclohexane mixtures. The product, m-hexadecyloxyphenyl-p-nitrophenylbenzylhydrazone (1A) was crystallized from ligroin at -78° C. (mp 77°-78° C.).

\*p-Nitrophenylbenzylhydrazone bromide was prepared from the p-nitrophenyl hydrazone of benzaldehyde as described in Tetrahedron, 28, 5903 (1972) and J. Chem. Soc., Perkin II, 1422 (1973).

**Rearrangement of the benzylhydrazone:**

The hydrazone (1A) (4 g, 7.8 mmol) was heated under nitrogen at 210° C. for 4 hours. The resulting rearranged product, 3-hexadecyloxy-3'-nitrodiphenyl-

N'-benzohydrazide (1B) (mp 74°-75° C.), was recrystallized from acetonitrile.

**Synthesis of the sulfonohydrazide (Compound 1):**

The hydrazide (1B) (2.5 g, 4.4 mmole) was added to 50 percent sodium hydride dispersion (1 g, 20 mmol) in tetrahydrofuran (75 ml) under nitrogen. The resulting dark red solution was cooled in an ice bath and dye sulfonyl chloride (3 g, 5.2 mmol)\*\* was added. The reaction mixture was warmed to room temperature (22° C.) overnight and treated with water (3 ml) followed by 1N sodium hydroxide (10 ml). After 30 minutes, the reaction mixture was poured over ice and hydrochloric acid and the resulting red precipitate was purified by silica gel column chromatography eluting with acetic acid, ethyl acetate/cyclohexane mixtures and trituration with methanol to yield 2.5 g, (58 percent) of the sulfonohydrazide product, Compound 1.

\*\*The dye sulfonyl chloride was prepared as described in Example 3 of U.S. Pat. No. 3,932,380 with the exception that the coupling reaction to form the dye was carried out prior to the reaction to unite the dye moiety to the carrier moiety of the present invention.

**Synthesis 2**

The schematic representation presented below describes preparation of positive RDR Compound 1 by the following sequence:



-continued



## Synthesis of hydrazone ester:

Ethyl- $\alpha$ -bromoglyoxylate-p-nitrophenylhydrazone (5 g, 15.8 mmol)\* and m-hexadecyloxyphenol (5.3 g, 15.8 mmol) were stirred together in a mixture of dichloromethane (100 ml) and water (20 ml) containing potassium hydroxide (1 g, 17.8 mmol). After 30 minutes, additional dichloromethane (200 ml) was added. The reaction was neutralized with 10 percent hydrochloric acid and the mixture was then dried over anhydrous magnesium sulfate. Purification by silica gel chromatography, eluting with dichloromethane/cyclohexane mixtures, and crystallization from ligroin yielded ethyl- $\alpha$ -hexadecyloxyphenylglyoxylate-p-nitrophenyl hydrazone (2A) (mp 99°–100° C.).

\*Ethyl  $\alpha$ -bromoglyoxylate p-nitrophenylhydrazone was prepared as described in JACS, 68 589 (1951).

Rearrangement and hydrolysis of the nitrophenyl hy-

acid and the red precipitate that formed was collected and purified by silica gel chromatography. This material was identical to the sulfonohydrazide product synthesized in 1C.

\*\*Prepared by a method described above in Synthesis 1.

## Synthesis 3 - Blocked Compound 13

Positive RDR Compound 1 (1.2 g, 1.2 mmole) was reacted with mono-(phthalimidomethyl)-2,2-dimethyl succinoyl chloride (1.5 g) in dichloromethane (50 ml) containing pyridine (5 equivalents). After stirring overnight at room temperature (22° C.) additional dichloromethane (50 ml) was added, followed by washing with 10 percent hydrochloric acid and drying over anhydrous magnesium sulfate. Purification by silica gel column chromatography yielded blocked RDR Compound 13 having the structural formula:



## drazone ester:

The hydrazone ester (2A) (22 g) was heated at 210° C. for 30 minutes under nitrogen. The resulting rearranged oily product (2B), which solidified upon standing, was refluxed overnight in ethanol (75 ml) containing concentrated hydrochloric acid (5 ml). Upon cooling in an ice bath, the yellow solid that formed was collected and recrystallized from acetonitrile to yield (82 percent) N-3-hexadecyloxyphenyl-N-4-nitrophenylhydrazine.HCl (2C).

## Synthesis of the sulfonohydrazide (Compound 1):

2C. The hydrazine (2C) (1 g, 2 mmol) and the dye sulfonyl chloride (1.2 g, 2 mmol)\*\* was stirred together in pyridine (20 ml) for 3 hours at room temperature (22° C.). The reaction was poured onto ice and hydrochloric

55

60

## EXAMPLE 1

To illustrate imaging and rate of dye release of sulfonohydrazide compounds of this invention, as compared with a prior art compound, the following integral imaging receiver elements were prepared by coating the described layers, in the order recited, on a transparent poly(ethylene terephthalate) support. Coverages are in (g/m<sup>2</sup>), and all parts, percents and ratios are by weight, unless otherwise specified:

1. image-receiving layer of poly(styrene-co-N-vinylbenzyl-N-benzyl-N,N-dimethylammonium chloride-co-N-vinylbenzene) (99:99:2 mole ratio) (2.3) and gelatin (2.3);

2. reflecting layer of titanium dioxide (19) and gelatin (3.0);

3. opaque layer of carbon black (1.9) and gelatin (1.2);

4. imaging layer of green sensitive negative silver bromoiodide emulsion (1.3 Ag), magenta redox dye releasing compound (0.27 mmol/m<sup>2</sup>) as identified in Table 1, incorporated reducing agent\* (0.48 mmol/m<sup>2</sup>) and gelatin (2.1);

\*The incorporated reducing agent in layer 4, which has the following structural formula, was dispersed in N,N-diethylauramide solvent at a 2:1 agent:solvent ratio:



5. overcoat layer of gelatin (0.55) and bis(vinylsulfonyl)methyl ether at 1.25 percent of the total gelatin weight.

Cover sheets were prepared by coating the following layers, in the order recited, on a poly(ethylene terephthalate) film support:

(1) acid layer comprising poly(n-butyl acrylate-co-acrylic acid) (30:70 weight ratio equivalent to 140 meq. acid/m<sup>2</sup>); and

(2) timing layer comprising a 1:1 physical mixture of the following two polymers coated at 4.8 g/m<sup>2</sup>:

(a) poly(acrylonitrile-co-vinylidene chloride-co-acrylic acid) wt. ratio 14:79:7; and

(b) a lactone polymer, partially hydrolyzed and 1-butanol transesterified poly(vinyl acetate-co-maleic anhydride) (ratio of acid/butyl ester 15:85).

Two viscous processing compositions were prepared:

|                                                     | Composition A      | Composition B |
|-----------------------------------------------------|--------------------|---------------|
| Potassium hydroxide                                 | 51. g/l (of water) | 51. g/l       |
| 4-Hydroxymethyl-4-methyl-1-p-tolyl-3-pyrazolidinone | 4.0 g/l            | —             |
| Carboxymethylcellulose                              | 50. g/l            | 57. g/l       |
| Potassium bromide                                   | 10. g/l            | —             |
| Sodium sulfite                                      | 2.0 g/l            | 2.0 g/l       |
| Ethylenediamine tetraacetic acid (disodium salt)    | 7. g/l             | 10. g/l       |
| Carbon                                              | 172 g/l            | —             |

Each integral image-receiving (IIR) element was exposed to a graduated density test object to yield a full-scale D-max/D-min image. The exposed elements were processed using viscous processing Composition A contained in a pod. The processing composition was spread between an IIR and a cover sheet using a pair of juxtaposed rollers to provide a fluid gap of 75  $\mu$ m. After three hours the Status A green density of the receiver side of the IIR was read to obtain the D-max and D-min values tabulated below.

TABLE

| RDR         | Image Discrimination |          |
|-------------|----------------------|----------|
|             | Dmin/Dmax            | $\Delta$ |
| Compound 1  | 0.22/1.4             | 1.18     |
| Compound 13 | 0.20/2.0             | 1.80     |

TABLE-continued

| RDR        | Image Discrimination |          |
|------------|----------------------|----------|
| Prior Art* | Dmin/Dmax            | $\Delta$ |
|            | 0.36/1.2             | 0.84     |

\*Sulfilimine dye releasing compound of the type disclosed in U.S. Pat. No. 4,369,243 having the same releasable magenta dye moiety as Compound 1:



15 As the data in the above Table indicate, improved image discrimination is obtained for the compounds of this invention as compared with the sulfilimine RDR compound of the prior art. Comparable dye release rates were obtained for all three RDR compounds.

20 This invention has been described in detail with particular reference to preferred embodiments thereof. However, it will be apparent that variations and modifications can be effected within the spirit and scope of the invention.

25 What is claimed is:

1. A photographic element comprising a support having thereon at least one photosensitive silver halide emulsion layer and also comprising, in said silver halide layer or in a layer adjacent thereto, a nondiffusible N,N'-di aromatic carbocyclic or aromatic heterocyclic sulfonohydrazide compound, or a precursor thereof, capable of releasing a diffusible photographically useful group wherein at least one of said aromatic groups comprises a nitro substituent in the 2- position or in a position conjugated thereto.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635

4. A photographic element according to claim 3 wherein at least one ring completed by Z is substituted with a straight chain alkyl or alkoxy group having from 1 to about 30 carbon atoms; an aryl group having from 6 to about 30 carbon atoms; a halogen atom; a carbamoyl group having the formula  $-\text{CON}(\text{R}^2)_2$  or a sulfamoyl group having the formula  $-\text{SO}_2\text{N}(\text{R}^2)_2$ , where each  $\text{R}^2$  independently represents a hydrogen atom; an alkyl or an alkoxy group having from 1 to about 30 carbon atoms or an aryl or an aryloxy group having from 6 to about 30 carbon atoms.

5. The photographic element according to claim 2 wherein a ballast group is substituted on at least one ring completed by Z.

6. The photographic element according to claim 5 wherein the ballast group has at least 8 carbon atoms.

7. The photographic element according to claim 2 wherein PUG is a dye or a dye precursor compound.

8. The photographic element according to claim 2 wherein PUG is a development inhibitor, a development accelerator, a bleach inhibitor, a bleach accelerator, a coupler, a developing agent, a silver complexing agent, a fixing agent, a toning agent, a hardening agent, a tanning agent, a fogging agent, an antifogging agent, a chemical sensitizing agent, a spectral sensitizing agent or a desensitizing agent.

9. The photographic element according to claim 2 wherein J is substituted in the 2- position of said carbon cyclic or heterocyclic ring.

10. The photographic element according to claim 2 wherein J is substituted in the 4- position of said carbon cyclic or heterocyclic ring.

11. The photographic element according to claim 1 wherein said nondiffusible compound is:

5

10

20

25

30

35



12. The photographic element according to claim 1 wherein said nondiffusible compound is:



13. A photographic assemblage comprising:

- (a) a photographic element according to any of claims 1 to 12;
- (b) a dye image-receiving layer; and
- (c) an alkaline processing composition with means for discharging same within said assemblage; said assemblage also comprising a silver halide developing agent.

\* \* \* \* \*

40

45

50

55

60

65